

## UNITED STATES PATENT OFFICE

2,176,668

## SILVER PLATING PROCESS

Birger Egeberg and Nathan Promisel, Meriden, Conn., assignors to International Silver Company, Meriden, Conn., a corporation of New Jersey

No Drawing. Application February 10, 1938.  
Serial No. 189,766

2 Claims. (Cl. 204—16)

This invention relates to electrodeposits of silver and similar metals, including silver alloys, and to a process of electrodeposition thereof.

This application is a continuation in part of our co-pending application Serial No. 70,396, filed March 23, 1936, now Patent No. 2,110,792.

In the present accepted commercial practice of electroplating silver coatings, the standard bath is composed of silver cyanide, an excess of alkali cyanide over that required to dissolve the silver cyanide, alkali carbonate and water. Through this solution an electric current of suitable characteristics is passed, the current passing into the solution through silver anodes of high purity, through the solution depositing silver on the articles to be plated which constitute the cathodes, and then out of the bath through the cathodes. Under proper conditions of current, temperature, agitation and maintenance of a proper concentration of the electrolyte, a crystalline, non-lustrous, matte white deposit of silver may be secured at the cathode. Buffing or burnishing, sometimes both, of such a deposit is, therefore, necessary to secure a bright surface. This buffing and burnishing is costly and wasteful and accordingly highly undesirable. It is, therefore, common practice to add to the above plating bath a brightener which will give the deposit, as it is made in the bath, a slightly lustrous appearance. For producing such a deposit, carbon-disulphide has been proposed and used commercially for nearly 100 years. A number of other brighteners have been also proposed such as gums, sugars, sodium thiosulphate, tellurium and selenium compounds and others. The only one in extensive commercial use, however, is carbon-disulphide and the other proposed brighteners have never come into extensive commercial use.

Carbon-disulphide although known and used for nearly a century has certain well-recognized disadvantages which may be briefly summarized as follows: Even under the best conditions the deposit is not satisfactory and frequently lacks any appreciable luster. It is, moreover, usually not uniform over the entire plated surface unless extreme precautions are taken. The deposit is sensitive to plating conditions in that the quantity of carbon-disulphide present, the current density, temperature, agitation and solution composition must all be adjusted and maintained within closely balanced limits. The carbon-disulphide limits are far narrower than required by the other components of the solution,

namely, the silver cyanide, alkali cyanide, carbonate and water. One difficulty in maintaining the proper quantity of carbon-disulphide present is that it is volatile at room temperature and this, in addition to its disappearance due to electrolysis, causes it to varnish rapidly from the solution making frequent additions necessary. Consequently, the precautions which have to be taken in dealing with this material are numerous. It is a fact that where many individual plating solutions including carbon-disulphide are used, even with the best of control, there are always certain solutions which perform unsatisfactorily and from which dull deposits are obtained, and even in solutions giving semi-lustrous deposits, there are always variations in appearance from vat to vat and even from section to section on the same article. In general, in employing this material, trial-and-error methods of plating have to be employed to secure the semi-lustrous deposits. Departure from conditions so determined may result in deposits the luster of which is actually inferior to those obtained from solutions containing no carbon-disulphide whatsoever. In addition, we have found with carbon-disulphide that only a relatively thin plating of semi-lustrous character can be obtained, in that, with increasing thickness of the deposit, the deposit changes from the semi-lustrous appearance to, eventually, a dull white appearance.

The principal object of the present invention accordingly is to provide a deposit or coating of silver that has as deposited an inherent, smooth, uniform, highly lustrous character even for the thickest commercial coatings. Another object of the invention is to provide a process for the production of such a deposit or coating which will do away with at least some of the objections to carbon-disulphide and other brighteners heretofore employed.

In accordance with our invention we have found that highly lustrous deposits or platings of silver may be produced under proper conditions of ingredient proportions and other characteristics of the solution and current employed, by electrolyzing a cyanide silver bath containing silver cyanide, alkali cyanide, and alkali carbonate in the presence of a brightener, comprising any of the group of chemical compounds represented by the formula



where  $X$  is a member of the group consisting of  $NH_2$  and substituted  $NH_2$  in which the substituents for hydrogen are methyl, ethyl, acetyl or  $NH_2$ . When  $X$  is  $NH_2$  the formula represents 5 urea



10 so that the remaining compounds above noted and embraced by the general formula, are substituted ureas. These compounds are such as not to produce ammonia since we find that the production of ammonia in our electrolytic baths 15 interferes with the proper luster.

The proportions of the brightener may vary from small amounts, in the neighborhood of a few grams per liter, to large amounts for example 100 g./l., depending upon the particular substance 20 and the attendant conditions. By proper adjustment of the plating conditions a silver deposit is secured superior in luster to any such deposits or coatings heretofore produced. The deposits and plating bath also have to a much 25 less extent the disadvantages enumerated above for carbon-disulphide and in some cases these disadvantages are completely eliminated.

The following is a preferred example of a plating bath in accordance with the invention employing urea 30



35 as a brightener, and a preferred method of using the same. The electrolytic bath contains

|                        |       |    |
|------------------------|-------|----|
| Silver cyanide         | grams | 25 |
| Potassium cyanide      | do    | 45 |
| 40 Potassium carbonate | do    | 20 |
| Urea                   | do    | 45 |
| Water                  | liter | 1  |

At a temperature of 80° F. lustrous silver deposits may be obtained at a current density of 45 6 amperes per sq. ft. of cathode surface.

Generally similar proportions and operating conditions are suitable where any of the other brighteners above noted are substituted for urea. The baths may be used immediately upon being prepared but we ordinarily prefer to allow them to age for two or three days before use.

The above mentioned brighteners are substantially non-volatile, and the deposits resulting from their use are substantially uniform and approach mirror brightness. Being of such high 10 luster they require little or no polishing. With these substances the current density, temperature, agitation and solution composition may be varied to the same extent as these factors vary in ordinary plating practice and it is not necessary, as in the case of carbon-disulphide, to adopt 15 any extreme precautions to produce the deposit. These materials may be consumed during electrolysis to some extent but by no means as rapidly as carbon-disulphide, and in any case their replenishment is easy to take care of. The range of 20 concentration of the materials as noted is not very critical and accordingly the control of the concentration is not difficult.

25 We claim:

1. A process for the electrodeposition of silver which comprises: electrolyzing a silver cyanide plating bath containing a brightener having the chemical formula



where  $X$  is a member of the group consisting of 35  $NH_2$  and substituted  $NH_2$  in which the substituents for hydrogen are methyl, ethyl, acetyl or  $NH_2$ , to form a bright deposit of silver therefrom.

2. A process for the electrodeposition of silver which comprises electrolyzing a silver cyanide 40 plating bath containing urea as a brightener to form a bright deposit of silver therefrom.

BIRGER EGEBERG.  
NATHAN PROMISEL.

45